

No. 781,914.

PATENTED FEB. 7, 1905.

J. S. SEAMAN.

MANUFACTURE OF CHILLED CASTINGS.

APPLICATION FILED MAY 23, 1904.

FIG.1.



FIG.2.



WITNESSES:

Herbert Bradley.  
Fred Kirchner.

INVENTOR

Joseph S. Seaman,  
by Christy & Christy, Atty's

## UNITED STATES PATENT OFFICE.

JOSEPH S. SEAMAN, OF PITTSBURG, PENNSYLVANIA.

## MANUFACTURE OF CHILLED CASTINGS.

SPECIFICATION forming part of Letters Patent No. 781,914, dated February 7, 1905.

Application filed May 23, 1904. Serial No. 209,310.

*To all whom it may concern:*

Be it known that I, JOSEPH S. SEAMAN, a citizen of the United States, residing at Pittsburgh, in the county of Allegheny and State of Pennsylvania, have invented or discovered certain new and useful Improvements in the Manufacture of Chilled Castings, of which improvement the following is a specification.

As is well known by those skilled in the art, not only the depth, but also the hardness of the chill on a roll or other article, depends upon the rapidity with which heat is carried away from the molten metal and the efficient persistence of this cooling action. The contraction of the molten metal during cooling and solidification and the expansion of the chill-ring when heated produce such a separation of the chill-ring and the cast metal that the former will not act by conduction to cool the cast metal, and the heat retained in the casting by reason of the heating of the chill-ring and its failure to carry away the heat will produce an annealing or softening effect on the chill produced by the first contact of the molten metal with the ring.

The present invention has for its object the employment of a chill-ring which will act effectively during the initial cooling of the metal, at which time the contraction is greatest, and the substitution of a second and preferably slightly smaller chill-ring for the first, whereby the article will be subjected to a secondary chilling action, which will be more continuing than the first chilling, and all annealing or softening action avoided.

The invention is hereinafter more fully described and claimed.

In the accompanying drawings, forming a part of this specification, Figure 1 is a sectional elevation of a mold for casting rolls, a casting being shown in position in the mold; and Fig. 2 is a similar view showing the parts after the first chill-ring has been removed and another ring placed in position.

In the practice of my invention the mold as regards the drag 1, chill-ring 2, and runner 3 are constructed in the usual or any suitable manner. The cope 4 may be constructed as is common in the art to permit the

chill-ring being drawn up outside of it, or, and 50 as is preferable, the cope is made in two vertical sections separated from each other by a thin metal ring 5. The matrices for the roll-neck wabbler and sinker-head are formed of clay within the ring 5, which has an external 55 diameter less than the internal diameter of the chill-ring 2. The space between the ring 5 and the cope-frame 4 is filled with a material such as sand, which will not cake or harden 60 when heated.

After the mold has been formed in the manner stated the metal is teemed in through the sprue, as is customary. The molten metal on coming into contact with the chill-ring is cooled and hardened. As the heat is conducted away from the metal by the chill-ring the latter will expand by reason of the heat absorbed, and the casting will contract. These opposite movements will so separate the casting and the chill-ring, that the latter will no 70 longer act with the desired efficiency. This loss of efficiency is due not only to the separation of the casting and chill-ring, but also to the heating of the chill-ring by the molten metal, so that the chill formed by the first contact of the molten metal with the chill-ring will 75 be softened by the annealing of the retained heat. As soon as this separation of the casting and the chill-ring has taken place and the shell of solidified metal forming the exterior of 80 the casting has become sufficiently rigid to prevent deformation of the casting when the chill-ring is removed the cope-frame and the material between it and the ring 5 are removed and the chill-ring 2 stripped off the casting. A second chill-ring 2<sup>a</sup>, preferably of slightly less diameter than the ring 2, is slipped down onto the casting. As this ring is cold and will come into direct contact with the surface of the casting, a second chilling action will occur 90 and will continue for a longer time, as the contraction of the casting at this stage is not as rapid as at first, nor will the chill-ring 2<sup>a</sup> be heated and expanded as rapidly.

I claim herein as my invention—

1. As an improvement in the art of manufacturing chilled castings the method herein described which consists in casting the metal

against a chill, removing the latter and substituting a second chill therefor, substantially as set forth.

2. As an improvement in the art of manufacturing chilled rolls, the method herein described which consists in casting the molten metal in contact with a chill-ring, permitting the formation of a rigid shell on the casting,

removing the chill-ring and substituting another therefor, substantially as set forth. <sup>10</sup>

In testimony whereof I have hereunto set my hand.

JOSEPH S. SEAMAN.

Witnesses:

DARWIN S. WOLCOTT,  
F. E. GAITHER.